

July 15, 1952

F. W. WOODMAN ET AL

2,603,594

METHOD OF ELECTROLYTICALLY PRODUCING MANGANESE

Filed May 13, 1947

*Fig. 1.*



*Fig. 2.*



*Fig. 3.*



INVENTORS  
FRANK W. WOODMAN &  
JAN MAX CROWELL

By  
Stebbins, Blenko & Webb.  
Atty.

## UNITED STATES PATENT OFFICE

2,603,594

METHOD OF ELECTROLYTICALLY  
PRODUCING MANGANESE

Frank W. Woodman, Maplewood, La., and Jan M. Crowell, Brisbane, Calif., assignors to Vanadium Corporation of America, New York, N. Y., a corporation of Delaware

Application May 13, 1947, Serial No. 747,672

6 Claims. (Cl. 204—105)

1

This invention relates to new and useful improvements in methods and apparatus for producing electrolytic manganese. The present application is a continuation-in-part of our application Serial No. 439,530 filed April 18, 1942, now abandoned.

In the accompanying drawings:

Figure 1 illustrates, in a diagrammatic manner, a cell for electro-depositing manganese according to prior known methods;

Figure 2 illustrates, in a diagrammatic manner, a cell for electrodepositing manganese according to our method; and

Figure 3 is a perspective view of one of the anode compartments of the cell shown in Figure 2.

In the electrodeposition of manganese from platable manganese solutions, principally sulphate and chloride baths have been used; however, the usual solution employed is manganese sulphate, but manganese sulphate solution cannot be employed alone because immediately upon depositing out some of the manganese, the solution becomes alkaline around the cathode and due to this alkaline condition, basic hydrated manganese salts precipitate. The principal salt is believed to be manganese hydroxide and where this term is used in this specification it is intended to include all such basic hydrated compounds. For this reason the manganese solution always has ammonium sulphate added to it, which serves the purpose of preventing the precipitation of manganese hydroxide. The higher the pH of the solution, the greater is the tendency of manganese hydroxide to precipitate. Accordingly, where high pH value solutions are employed, it is necessary to employ relatively large amounts of ammonium sulphate to prevent this objectionable precipitation of manganese hydroxide. Similarly, ammonium chloride may be employed in manganese chloride baths to prevent the precipitation of manganese hydroxide.

The electrodeposition of manganese presents a distinctly different problem from that involved in electrodepositing certain other metals where compartment cells may beneficially be used, such as cadmium or nickel. Nickel, for example, does not have the objectionable property of forming hydrated oxides, and accordingly in the electrodeposition of nickel from solution it is not necessary to employ ammonium sulphate along with nickel sulphate. Thus in depositing nickel no problem is involved as to the relative proportions of nickel sulphate and ammonium sulphate, since ammonium sulphate need not be employed.

2

Successful and economical deposition of manganese from solutions must be carried out under very carefully controlled conditions in which for best results the pH value, concentration of manganese and the temperature are regulated according to the current density used.

The reactions occurring in the manganese electrolytic cell are as follows:

Anode reactions:

- 10 (1)  $2H_2O = O_2 + 4H$   
 (2)  $MnSO_4 + O_2 = MnO_2 + SO_4$   
 (3)  $2H + SO_4 = H_2SO_4$

Cathode reactions:

- 15 (4)  $MnSO_4 = Mn + SO_4$   
 (5)  $2H_2O = H_2 + 2OH^-$   
 (6)  $2H + SO_4 = H_2SO_4$

Manganese metal possesses a very low hydrogen overvoltage. Therefore the pH value of the solution surrounding the cathode must be carefully regulated as otherwise, re-solution of the deposited manganese by the sulphuric acid generated at the anode would occur. To prevent 25 the acid at the anode from coming in contact with the manganese metal deposited on the cathode, a diaphragm is interposed between the two electrodes.

Interposing the diaphragm between the electrodes presents a major problem, i. e., control of the catholyte pH. It is well known that manganese in alkaline solutions will precipitate as the hydroxide and, if such precipitation occurs around the cathode, it will contaminate the manganese deposit and will eventually cause the deposition of metallic manganese to cease. Ammonium sulphate is used in order to protect the cathode manganese from precipitated manganese hydroxide because ammonium sulphate will prevent its precipitation although the hydroxide may be present in solution. The amount of ammonium sulphate in solution which is required to prevent the precipitation of manganese hydroxide depends on the pH of the solution in the cathode compartment. The higher the pH of the catholyte, the more ammonium sulphate is required and vice versa.

Heretofore, in the electrodeposition of manganese the practice has been to place each individual cathode in a compartment with a diaphragm as an integral part thereof (see Electrolytic Manganese, J. Koster et al., Engineering & Mining Journal, vol. 137, page 510). When a cathode is surrounded by a relatively small diaphragm, the volume of solution contained around

each cathode is small and is therefore subject to radical changes in pH value, concentration of manganese, and temperature. For this reason, in carrying out the electrodeposition of manganese in accordance with prior methods in which the cathodes were enclosed in diaphragms, it was essential that the ammonium sulphate concentration of the catholyte be kept at a relatively high amount in order to insure the presence of sufficient ammonium sulphate to largely prevent the precipitation of manganese hydroxide when the pH of the catholyte fluctuated widely.

Fig. 1 illustrates in a diagrammatic manner the previously used method of electrodepositing manganese where the individual cathodes were surrounded by diaphragms. In this figure, tank 2, containing a solution 3 of manganese sulphate and ammonium sulphate is provided with alternately arranged anodes 4, and cathodes 5. Each individual cathode is surrounded by a diaphragm 6. The solution is fed to the individual cathode compartment 6 as indicated by the arrows 7. Since each individual cathode compartment is of relatively small volume, the individual feeds must be very accurately controlled and in spite of all such precautions the pH and other conditions of the catholyte in the individual compartments 6 varies radically in commercial operations. Accordingly, it is necessary to employ a large excess of ammonium sulphate to prevent precipitation of manganese hydroxide under widely varying conditions obtaining in the small catholyte compartments. A further objection to the old method was that the catholyte feed to each compartment (being small in amount) was not uniform, and therefore resulted in variable electrodeposition. Another difficulty was encountered in removing and replacing the cathode in the cathode compartment during the stripping operation. During the electrodeposition process a certain amount of salting occurs in the cathode compartment due to the usual limited precipitation in the cathode compartment of manganese hydroxide. The manganese hydroxide settles to the bottom of the cathode compartment and contacts the lower portion of the manganese which has been deposited and contaminates the deposit as well as causing re-solution of the already deposited metal.

In accordance with our invention we place each of the individual anodes within a compartment and suspend the anodes so compartmented in an electrolytic tank between cathodes freely suspended in the tank. This system has certain very valuable features and is illustrated diagrammatically in Fig. 2. As shown therein, a tank 10 containing an electrolyte 11 is provided with a plurality of alternately arranged anodes 12 and cathodes 13. Each of the anodes is surrounded by a diaphragm 14, whereas the cathodes are freely suspended in a single body of solution 15 of large volume as compared with the volume of any individual anode compartment 14. The catholyte compartment may be fed by a single feed indicated by the reference numeral 16, as contrasted with the large number of small feeds 7 required in the arrangement shown in Fig. 1.

The arrangement shown in Fig. 2 allows a plurality of cathodes to be suspended in one relatively large body of catholyte, to which catholyte may be added fresh cell feed through one or more ports. These ports may be controlled automatically by floats or other known liquid-level apparatus much more expeditiously than

could be accomplished by the previous practice, since the cathode compartment is a single body. In one example of commercial practice according to the old method (see Fig. 1), 27 cathode compartments designated by reference numeral 6 were employed. Since each cathode compartment was divided in two by the cathode, this in effect meant that the cell contained 54 separate cathode compartments, each requiring an individual feed. By reference to Fig. 2 it will be seen that the entire cell may be fed by a single feed 16 since the catholyte forms a single body. This single body is of very large volume compared with any one of the individual compartments 14, and accordingly conditions in the catholyte compartment 15 may be very accurately controlled.

Another advantage of the arrangement shown in Fig. 2 is that the removal and replacement of the cathodes during stripping operations is facilitated. In previous practice the cathodes were placed in grooved guides within the cathode compartment frames. The electrodeposited metal sometimes wedged the cathode into the frame and the removal of the cathode damaged either the cathode, the frame, or both. These disadvantages are overcome in the arrangement according to Fig. 2, in which the cathodes are freely suspended in the catholyte, 15.

The replacement of each cathode in its frame had to be under delicate control and had to be done manually. With the arrangement shown in Fig. 2, however, the cathodes can be removed and replaced in the tank mechanically because they do not have to be inserted in grooved frames in the tank but are simply suspended in the catholyte. A uniform catholyte composition is maintained around each cathode where formerly there were twice as many catholyte compositions to control as there were cathodes.

As previously stated, manganese hydroxide tends to precipitate from alkaline solutions at the cathode and according to prior practice it has been necessary to employ large amounts of ammonium sulphate to largely prevent this precipitation. It was necessary to employ large amounts of ammonium sulphate to cover wide fluctuations in pH and other conditions which occurred in cathode compartments of small volume. It will be seen that in the new arrangement shown in Fig. 2, the catholyte compartment 15 is of large volume as compared with the individual anode compartments 14 and for this reason the pH value and other conditions of the catholyte can be accurately controlled. Since there are no wide variations in the pH and other conditions of the catholyte, the amount of ammonium sulphate added can be accurately adjusted to approximately the quantity actually needed to practically prevent precipitation of manganese hydroxide. Such limited amount of precipitate as cannot be prevented accumulates at the bottom of the tank out of contact with the cathodes and is readily removable as contrasted with accumulation against the cathode at the bottom of the diaphragm as in Fig. 1. This means that less ammonium sulphate is required in the catholyte. It is to be noted that the solution fed to a manganese electrolytic cell is saturated with respect to manganese sulphate and ammonium sulphate. Therefore, since less ammonium sulphate is required in the catholyte, the concentration of ammonium sulphate in the feed can be decreased and the concentration of manganese sulphate in the feed can be increased. Higher concentrations of manganese sulphate in

the cell feed result in higher concentrations of manganese in the catholyte which permits the employment of higher current densities while still obtaining high current efficiencies.

It is known that processes of electrodepositing manganese operate more efficiently at low temperatures than at high temperatures due to the fact that decrease in temperature of the catholyte tends to increase the hydrogen over-voltage on manganese. In the old arrangement shown in Fig. 1, in which the cathodes were surrounded by diaphragms, it was impossible to place cooling coils in the individual catholyte compartments because of the small space available. Accordingly, cooling coils were placed in the anolyte compartment and the cooling of the catholyte was dependent upon heat transfer from the catholyte compartment through the diaphragm to the anolyte compartment. This was a very inefficient way of regulating the temperature of the catholyte. In the arrangement shown in Fig. 2, however, there is sufficient space in the catholyte compartment 15 for the reception of cooling coils which enable efficient cooling of the catholyte, whereby the efficiency of the electrodepositing operation is substantially increased. By efficiently cooling the catholyte, increased current densities have been made possible because increased current densities always are accompanied by more heat. Accordingly, the capacity of an electrolytic cell constructed in accordance with Fig. 2, having a large volume of catholyte and a small volume of anolyte is increased in two ways: (1) by increasing the current efficiency, and (2) by increasing the current density. The statement just made that the cell of Fig. 2 has a large volume of catholyte and a small volume of anolyte means, of course, that the catholyte has a volume greater than all of the anolytes combined.

During the electrodeposition of manganese the anolyte is more acid than the catholyte. It is necessary to prevent the more acid anolyte from diffusing into the less acid catholyte since otherwise the acid would dissolve the manganese which has been deposited. In the arrangement shown in Fig. 1 there is a large volume 8 of more acid anolyte and a small volume 9 of catholyte of higher pH. Thus the diffusion of the anolyte into the catholyte causes a substantial decrease in the pH of the catholyte. Referring to Fig. 2, however, the volume of more acid anolyte 14 is relatively small as compared with the volume of catholyte 15 of higher pH. Thus the diffusion of the anolyte into the catholyte does not cause any substantial decrease in the pH of the catholyte.

Referring now to Figures 2 and 3 of the accompanying drawings:

The cell proper comprises a tank 10 of suitable acid-resistant material constructed in accordance with the customs usually prevailing in the electrolytic industries. These tanks are conventionally rectangular with an open top, but having bottom, end, and side walls, one of the side walls, indicated by the reference character 19, appears in Fig. 2. One common practice is to fabricate the tanks of wood and line them with lead, but any suitable tank may be used so far as our invention is concerned.

Cathodes 13, which may be formed of any suitable metal, such as stainless steel or aluminum, are conventionally provided with wooden strips around their edges in order to eliminate the well known "edge" effect of electrolytic deposition. Our invention, however, is not primarily

concerned with the support for or details of the cathode.

The anodes 12 are suitably supported within the anode frame, to be described, and are preferably formed of a material which will inhibit the formation of manganese oxide, examples of such anodes being: (A) an alloy containing about equal proportions of lead and tin and a relatively small proportion, e. g. 2% to 4% of cobalt; or (B) lead-silver anodes containing a small amount, e. g. 1% to 2.5%, of silver. Instead of using anodes which themselves minimize the formation of manganese oxide, we may employ lead anodes and introduce sulphur dioxide or other reducing agent into the anode compartments to prevent the formation of manganese oxide at the anodes. An installation in accordance with our invention would of course involve the usual arrangement of a plurality of cells, with suitable generator equipment, bus bars along the cells, and connections to anodes and cathodes, none of which we deem essential to bring out clearly the details of our invention.

An anode frame 14 is shown in Fig. 3. The anode frame comprises cross pieces 18 which bridge the tank 10 and rest upon the upper edges of the tank sides 19. The frame has a bottom 20 and two side frame members 21 made of wood. A diaphragm 14a is supported on either side of the anode frame and is of suitable character for the purpose at hand. The diaphragm may be closely woven cloth such as heavy duck or canvas or in general any porous or semi-porous septum material which will permit migration of ions between the catholyte and anolyte. Shelton in Patent 2,119,560 and Koster et al. in Electrolytic Manganese, Engineering & Mining Journal, vol. 137, page 510, discuss suitable types of diaphragms for use in electrodepositing manganese. Thus it will be seen that the anodes are separately completely enclosed in a compartment, the walls of which comprise essentially a diaphragm, and the cathodes are all in one catholyte compartment comprising the entire remaining portion of the electrolytic tank.

In the operation of the cell, the cell feed is delivered continuously to the cathode compartment 15 through a pipe 16. Suitable valve means (not shown) may be provided to control the flow. Preferably the level of anolyte is kept only slightly below the level of the catholyte by suitably continuously withdrawing the anolyte from the separate compartments by suitable means, for example, by gravity through an overflow vent and drain line 22 at the same rate as platable manganese solution is fed to the tank 10. The catholyte flows to the anolyte compartment because of the lower hydraulic head by seepage, percolation, diffusion, or dialysis through the diaphragm, or vents such as those shown at 23 in Fig. 3 may be used to provide for direct liquid flow between the two compartments. It will be seen that the catholyte flows directly into the individual anolyte compartments while all of the catholyte is maintained in the tank 10. Thus the catholyte at no time has access to air in amounts sufficient to form an appreciable quantity of basic hydrated manganese salts in the catholyte. The flow of catholyte within the tank is in a relatively quiescent manner, as can be seen from the fact that the catholyte merely seeps through the diaphragm into the anolyte compartments or flows through the port 23 which is located only at a slightly higher level than the vent 22 and accordingly there is not sufficient agitation of the

catholyte to cause the air which contacts the surface of the catholyte to form an appreciable quantity of basic hydrated manganese salts in the catholyte.

The details of construction of the cell are not of prime importance in the practice of our invention, and the cell details as shown may be modified extensively within the scope of our invention. Any usual means for supporting the anodes and cathodes in the tank, and connecting them into the electrical circuit, may be employed. In general, this may involve the use of negative and positive bus-bars at opposite sides of the cell, with anode and cathode bus-bars running transversely of the cell, and connected to (and in many installations supported at one side by) the positive and negative bus-bars, respectively. As a rule the ends of the anode and cathode bus-bars opposite to those engaging the positive and negative bus-bars are supported by the opposite top edge of the tank. This usual construction or other suitable construction for supporting the anodes and cathodes may be used with our invention, but this has not been shown in the drawing since it is not a part of our invention. We merely wish to point out that our invention is adapted for use with any usual types of installation with little or no change except in so far as the diaphragm arrangement is concerned.

The following are examples illustrating the results obtained according to previously known methods and other examples illustrating our invention. Example 1 is illustrative of results obtained according to prior investigators as reported in Bureau of Mines Report of Investigations, R. I.-3406, by S. M. Shelton and others.

#### Example 1

The cell contained alternately arranged anodes and cathodes, each cathode being enclosed in an individual diaphragm. The feed solution consisted of 200 grams per liter of ammonium sulphate, and 25 grams per liter of manganese. The catholyte contained about 10 grams per liter of manganese and had a pH of 9-9.2. The plating was done at a current density of 18-20 amps. per sq. ft. at a temperature of about 31° C. The current efficiency was about 50%.

#### Example 2

Example 2 illustrates the present invention. The plating tank contained alternately arranged anodes and cathodes, each anode being enclosed in a diaphragm; the anodes were lead-silver anodes and the cathodes were chromium-containing steel. The feed solution contained 171 grams per liter of ammonium sulphate and 42.3 grams per liter of manganese. This is a ratio by weight of about 4.0 parts of ammonium sulphate to 1 part of manganese. The catholyte had a pH value between 6.5 and 7.0 and contained 25 grams of manganese per liter. The current density ranged from 40 to 70 amps. per sq. ft. and the current efficiency was between 60.2% and 64%. The strip was 17.3 grams per liter of manganese.

#### Example 3

This example also is illustrative of our invention, each anode being enclosed in a diaphragm. The feed solution contained 130-135 grams per liter of ammonium sulphate and 35 grams per liter of manganese. This is a ratio by weight of about 3.7 parts of ammonium sulphate to 1 part of manganese. The catholyte contained 13 grams

per liter of manganese and had a pH of 8.2-8.4. The plating was done at a cathode current density of 45-50 amps. per sq. ft. with a resulting current efficiency ranging between about 60% and 65%.

The advantages of our process can be seen from a comparison of Examples 2 and 3 (which illustrate our process), with Example 1 (which is illustrative of the prior art). In our examples, current densities from 40 to 70 amps. per sq. ft. were employed as contrasted with current densities of 18 to 20 amps. per sq. ft. in the prior practice. In our process the concentration of manganese in the catholyte was from 13-25 grams per liter as compared with 10 grams per liter in Example 1. In our examples, 17 to 22 grams of manganese per liter were stripped as compared with 15 grams per liter in Example 1. The current efficiency in our examples was from 60% to 65% as contrasted with a current efficiency of about 50% in Example 1.

In carrying out our process, the current density may be as low as 18 amps. per sq. ft. or as high as 275 amps. per sq. ft. As the current density increases, the current efficiency generally decreases. The preferred current density is between 40 and 70 amps. per sq. ft. The pH may be between 2 and 9.2 but preferably is between 6 and 8.5. The manganese concentration in the catholyte may be between 8 and 75 grams per liter. The feed solution may contain between 25 and 100 grams per liter of manganese and between 25 and 200 grams per liter of ammonium sulphate.

The invention is not limited to the examples but may be otherwise embodied within the scope of the following claims.

We claim:

1. The method of electrolytically producing manganese metal, which comprises providing a body of platable manganese solution in a tank, continuously feeding a platable manganese solution to said body, passing a current of about 18-275 amperes per square foot between anodes and cathodes arranged in said body to cause manganese metal to plate on the cathodes, separating each anode from the cathodes by an individual diaphragm of such porosity that ions can migrate therethrough so as to provide a plurality of individual anolytes and a single catholyte having a volume greater than all of the anolytes combined, flowing the catholyte directly into the individual anolytes while maintaining all of the catholyte in the tank, and continuously withdrawing anolyte from the individual anolytes.

2. The method of electrolytically producing manganese metal, which comprises providing a body of platable manganese solution in a tank, continuously feeding a platable manganese solution to said body, passing a current of 18-275 amperes per square foot between anodes and cathodes arranged in said body to cause manganese metal to plate on the cathodes, separating each anode from the cathodes by an individual diaphragm of such porosity that ions can migrate therethrough so as to provide a plurality of individual anolytes and a single catholyte having a volume greater than all of the anolytes combined, flowing the catholyte directly into the individual anolytes while maintaining all of the catholyte in the tank, and continuously withdrawing anolyte from the individual anolytes at the same rate as platable manganese solution is fed to said body.

3. The method of electrolytically producing manganese metal, which comprises providing a body of platable manganese solution in a tank,

continuously feeding a platable manganese solution to said body, passing a current of 18-275 amperes per square foot between anodes and cathodes arranged in said body to cause manganese metal to plate on the cathodes, separating each anode from the cathodes by an individual diaphragm of such porosity that ions can migrate therethrough so as to provide a plurality of individual anolytes and a single catholyte having a volume greater than all of the anolytes combined, flowing the catholyte directly into the individual anolytes while maintaining all of the catholyte in the tank, and while preventing access of air in amounts sufficient to form an appreciable quantity of basic hydrated manganese salts, and continuously withdrawing anolyte from the individual anolytes.

4. The method of electrolytically producing manganese metal, which comprises providing a body of platable manganese solution containing ammonium sulphate and manganese sulphate, continuously feeding to said body a platable manganese solution containing about 25-200 grams per liter of ammonium sulphate and about 25-100 grams per liter of manganese, passing a current at a current density of about 18-275 amperes per square foot between anodes and cathodes arranged in said body to cause manganese metal to plate on the cathodes, separating each anode from the cathodes by an individual diaphragm of such porosity that ions can migrate therethrough so as to provide a plurality of individual anolytes and a single catholyte having a volume greater than all of the anolytes combined, flowing the catholyte directly into the individual anolytes while maintaining all of the catholyte in the tank, and continuously withdrawing anolyte from the individual anolytes.

5. The method of electrolytically producing manganese metal, which comprises providing a body of platable manganese solution containing ammonium sulphate and manganese sulphate, continuously feeding to said body a platable manganese solution containing about 25-200 grams per liter of ammonium sulphate and about 25-100 grams per liter of manganese in a ratio by weight of about 3.7 to 4 parts of ammonium sulphate to 1 part of manganese, passing a current at a current density of about 18-275 amperes per square foot between anodes and cathodes arranged in said body to cause manganese metal to plate on the cathodes, separating each anode from the cathodes by an individual diaphragm of such porosity that ions can migrate therethrough so as to provide a plurality of individual anolytes and a single

catholyte having a volume greater than all of the anolytes combined, flowing the catholyte directly into the individual anolytes while maintaining all of the catholyte in the tank, and continuously withdrawing anolyte from the individual anolytes.

6. The method of electrolytically producing manganese metal, which comprises providing a body of platable manganese solution containing ammonium sulphate and manganese sulphate, continuously feeding to said body a platable manganese solution containing about 25-200 grams per liter of ammonium sulphate and about 25-100 grams per liter of manganese in a ratio by weight of about 3.7 to 4 parts of ammonium sulphate to 1 part of manganese, passing a current at a current density of about 40-70 amperes per square foot between anodes and cathodes arranged in said body maintained at a pH between about 6 and 8.5 to separating each anode from the cathodes by an can migrate therethrough so as to provide a plurality of individual anolytes and a single catholyte having a volume greater than all of the anolytes combined, flowing the catholyte directly into the individual anolytes while maintaining all of the catholyte in the tank, and continuously withdrawing anolyte from the individual anolytes.

FRANK W. WOODMAN.  
JAN M. CROWELL.

#### REFERENCES CITED

The following references are of record in the file of this patent:

#### UNITED STATES PATENTS

| Number    | Name          | Date           |
|-----------|---------------|----------------|
| 496,863   | Craney        | May 9, 1893    |
| 1,375,631 | Haglund       | Apr. 1921      |
| 1,878,244 | Laury         | Sept. 20, 1932 |
| 2,112,691 | Crowder       | Mar. 29, 1938  |
| 2,119,560 | Shelton       | June 7, 1938   |
| 2,286,148 | Mantell       | June 9, 1942   |
| 2,320,773 | Fink          | June 1, 1943   |
| 2,439,805 | Hanley et al. | Apr. 20, 1948  |
| 2,456,196 | Jacobs et al. | Dec. 14, 1948  |

#### FOREIGN PATENTS

| Number  | Country | Date         |
|---------|---------|--------------|
| 666,431 | France  | Oct. 1, 1929 |

#### OTHER REFERENCES

Webster's International Dictionary, 2d edition unabridged, page 2283, Merriam Co. (1940).  
Bureau of Mines, Bulletin 463 (1946), pages 59, 55, 60, 61, 62, and 63.